

1

2,884,322

## EXTRACTION OF CYANIDABLE PRECIOUS METALS FROM CARBONACEOUS ORES

Norman Hedley and Howard Tabachnick, Stamford, Conn., assignors to American Cyanamid Company, New York, N.Y., a corporation of Maine

No Drawing. Application January 22, 1957  
Serial No. 635,136

5 Claims. (Cl. 75—105)

This invention relates to an improved method of recovering precious metals from carbon-containing ores.

The cyanidation of precious metal ores, such as gold and silver ores, is the standard method for recovering the precious metal values and under suitable conditions is highly efficient. However, there are ores which present serious problems. One type of ore is that containing carbon or carbonaceous impurities. Apparently, the carbon causes a reprecipitation of the dissolved gold and/or silver from their complex cyanide solutions. As a result when such ores are cyanided, recoveries suffer and in some cases cyanide consumption increases. As a result these carbonaceous ores were for many years considered as unsuitable for cyanidation.

Attempts have been made to overcome the difficulties by the addition of certain materials. For example, mineral oils, such as fuel oil, were described in the Dorfman Patent 1,411,326. The patentee was of the opinion that these mineral oils were adsorbed on the carbonaceous material and so presumably insulated it from contact with the dissolved precious metal complex cyanide. The hydrocarbon oil does, in fact, improve extraction, whether by reason of the suggested mechanism or for some other reasons, but there is a limit to the improvement which may be obtained and extractions of previous metal still leave much to be desired, although the fuel oil does help and as will be pointed out below may be used in conjunction with the other reagents to which the present invention relates.

Another solution to the problem is described in the Booth Patent 2,220,034 in which certain dyes are used. This process is a marked improvement and has been successfully used on some carbonaceous ores. The price of the dyes, however, is quite high, and there was therefore still left a demand for an equally efficient or more efficient process which uses cheaper material.

The present invention utilizes reagents belonging to five different groups of organic chemicals. The mechanism is not entirely understood, and it is not known why the different chemical classes operate. It is possible that there is some common characteristic or mechanism of reaction. It is also possible that each group behaves in a different manner. Except for the fact that the different groups are effective in producing better precious metal extraction, it is not known that they are in any sense equivalents or operate by the same reaction mechanism.

The first group of chemical compounds used in the present invention are aralkyl mercaptans which, of course, may exist in the normally strongly alkaline cyanidation pulps partly or wholly as the corresponding alkali or alkaline earth metal mercaptides. This group of compounds must have a larger number of aromatic carbon atoms than aliphatic carbon atoms. This is quite critical but the reason for this behavior is not known and, accordingly, this invention is not limited to the theory of why the reagents are sensitive to an excessive amount of aliphatic carbon atoms.

The second class of compounds are diaryldithiophosphoric acids which also exist as their salts in the strongly alkaline cyanidation pulps. The aryl radicals in the diaryldithiophosphoric acid may contain alkyl substituents.

In the case of this type of compound, however, there is a much greater tolerance for aliphatic carbon atoms but here again there is a very definite limit. The aliphatic carbon atoms must be not more than twice the number of aromatic carbon atoms.

The third class are diarylthioureas. Here again there is a limited tolerance for aliphatic carbon atoms but there should be more aromatic carbon atoms than aliphatic carbon atoms, the carbon atom of the thiourea itself being considered as neutral.

The fourth type of compound is a mercaptothiazole.

The fifth type of compound is an alkyl phenol, but here the presence of alkyl carbon atoms is essential, for phenol itself is not effective, and there does not appear to be any limitation on the number of aliphatic carbon atoms, mono- and polyalkyl phenols being very effective.

The amount of reagent used is not critical and ranges from a small fraction of a pound per ton of ore up to several pounds per ton. In the case of many of the compounds and with certain ores, amounts from 1 to 2 pounds per ton are very effective. Larger amounts may be used but no benefit is obtained when the amount greatly exceeds 2 or 3 pounds per ton. Consequently, it is desirable to use as little reagent as will give good extractions. Normally, however, the reagents are sufficiently cheap so that a small excess over the absolute minimum for any given ore is desirable to take care of the operating variations.

It is in no sense necessary that compounds of only one of the five classes be used. On the contrary, mixtures of more than one compound in the class, or of compounds belonging to more than one class, are equally effective and with certain refractory ores occasionally show some advantage. It is also possible to use the hydrocarbon oils, such as light fuel oils, with the reagents of the present invention. In some cases this permits the use of a somewhat smaller amount of the more expensive chemical. In other cases, for example with some very refractory ores, the result of the mixture is actually better. The present invention therefore contemplates the use of compounds belonging to one or more of the five classes enumerated above with or without fuel oil, or other hydrocarbon oil.

It is a very real advantage of the present invention that the reagents may be very crude. Within wide limits purity of the compound does not appear to be of any importance. It is thus possible to use crude compounds such as flotation-grade dithiophosphates, diarylthioureas, etc. These crude compounds are much cheaper than pure chemicals and, because they are just as effective, they are preferred for economical reasons.

The present invention is not limited to the use of inorganic cyanides in conjunction with the reagents of the five classes. On the contrary, excellent results are obtained when the cyanidation reagent is an alpha-hydroxynitrile, such as lactonitrile, mandelonitrile and the like. Very crude alpha-hydroxynitriles may be used such as the crude lactonitrile obtained as a dirty brown by-product from the production of acrylonitrile.

It should be noted that the aromatic groups in the substituted thioureas need not in all cases be linked to the nitrogen of the thiourea from a nuclear carbon atom.

Aralkyl groups such as benzyl are equally effective. It should be noted also that, particularly in the case of the modified mercaptans, the presence of inorganic substituents in the aryl groups such as halogens do not interfere with the effectiveness of the reagent. How-

ever, in general these inorganic substituents should be covalently linked, rather than electrovalently linked.

The invention will be described in conjunction with the specific examples which are typical in carbonaceous ores which are not amenable to ordinary cyanidation.

In each case the ore was ground to the fineness specified in the example, diluted with water to a pulp of approximately 25% solids, and subjected to cyanidation under otherwise standard conditions with 4.0 pounds per ton NaCN. In each case lime was added to produce an alkaline pH for optimum extraction. The pH's were of the order of 11. The other operations also follow standard cyanidation practice. In each case the pulp was filtered, washed and the solution then treated to extract the precious metals and assayed. Unless otherwise specified cyanidation time was 24 hours.

Because of the strong alkalinity of the conventional cyanidation pH used, the acidic reagents, such as the dithiophosphoric acids and also perhaps in the case of the mercaptans and the mercaptothiazoles, the actual compound exists in the form of its alkali salt. In the claims, therefore, the diaryldithiophosphoric acid will be expressed as the anion as it exists in combination with whatever cation is used in the alkali to produce the pH in question. The term "mercaptan" is used generically to include its salts.

#### Example 1

A Canadian ore from Canada assaying 0.311 oz. gold per ton and 1.82% carbon was ground to 91% —200 mesh and portions were cyanided for 48 hours. The results with the different added reagents and the blank appear in the following table.

| Reagent Used                                                       |                    | Residue Au, oz./ton | Extr. Au, Percent |
|--------------------------------------------------------------------|--------------------|---------------------|-------------------|
| Name                                                               | Amt. Used, lb./ton |                     |                   |
| Blank                                                              |                    |                     |                   |
| Di (2-naphthyl) dithiophosphoric acid                              | 2.0                | 0.306               | 1.0               |
| Mixture of Di cresyl dithiophosphoric acid and thiocarbanilide     | 2.0                | 0.085               | 72.9              |
| Ammonium di (2-naphthyl) dithiophosphate                           | 2.0                | 0.103               | 67.3              |
| 1-Benzyl-1-phenylthiourea                                          | 2.0                | 0.109               | 63.6              |
| Mixture of Di cresyl dithiophosphoric acid and an aromatic solvent | 2.0                | 0.157               | 52.3              |
|                                                                    |                    | 0.075               | 76.6              |

#### Example 2

A Canadian ore analyzing 0.313 oz. gold per ton and 1.12% carbon was ground to 93% —200 mesh and portions cyanided for 48 hours. The results with different reagents are shown in the following table.

| Reagent Used                                                   |                    | Residue Au, oz./ton | Extr. Au, Percent |
|----------------------------------------------------------------|--------------------|---------------------|-------------------|
| Name                                                           | Amt. Used, lb./ton |                     |                   |
| Blank                                                          |                    |                     |                   |
| Mixture of Di cresyl dithiophosphoric acid and thiocarbanilide | 2.0                | 0.288               | 4.0               |
| p-Isopropylbenzylmercaptan                                     | 2.0                | 0.060               | 81.1              |
| Dimethylbenzylmercaptan                                        | 2.0                | 0.085               | 73.4              |
| Mercaptomethylidimethylnaphthalene                             | 2.0                | 0.066               | 79.0              |
| 3,4-Dichlorbenzylmercaptan                                     | 2.0                | 0.099               | 70.2              |
| Zinc diethylphenyl dithiophosphate                             | 2.0                | 0.078               | 76.1              |
| Triisopropylbenzylmercaptan                                    | 2.0                | 0.103               | 66.9              |
| Dodecylbenzylmercaptan                                         | 2.0                | 0.217               | 31.8              |
|                                                                |                    | 0.210               | 29.3              |

It will be noted that alkylbenzylmercaptans having more alkyl carbon atoms than aromatic carbon atoms give very inferior results, although better than the blank alone.

The procedure of the above example was repeated using 4 lb./ton NaCN equivalent of crude lactonitrile with 2 lb./ton of a mixture of one part of a 6% solution of thiocarbanilide in technical grade di cresyl dithiophos-

75

phoric acid and one part of a crude aromatic hydrocarbon oil. The residue contains 0.058 oz./ton Au and the extraction was 82.2%.

#### Example 3

A Canadian ore analyzing 0.437 oz. gold per ton and 1.33% carbon was ground to 98% —200 mesh and portions were cyanided for 48 hours. The results appear in the following table.

| Reagent Used                                                                    |                    | Residue Au, oz./ton | Extr. Au, Percent |
|---------------------------------------------------------------------------------|--------------------|---------------------|-------------------|
| Name                                                                            | Amt. Used, lb./ton |                     |                   |
| Blank                                                                           |                    | 0.270               | 36.9              |
| p-Isopropylbenzylmercaptan                                                      | 2.0                | 0.055               | 88.2              |
| Mixture of Di cresyl dithiophosphoric acid and thiocarbanilide                  | 2.0                | 0.050               | 89.1              |
| Mixture of Di cresyl dithiophosphoric acid and an aliphatic hydrocarbon solvent | 2.0                | 0.039               | 91.2              |

#### Example 4

An ore from the Gold Coast analyzing 0.71 oz. gold per ton and 1.37% carbon was ground to 82% —200 mesh and portions cyanided. The results appear in the following table.

| Reagent Used                                                      |                    | Residue Au, oz./ton | Extr. Au, Percent |
|-------------------------------------------------------------------|--------------------|---------------------|-------------------|
| Name                                                              | Amt. Used, lb./ton |                     |                   |
| Blank                                                             |                    | 0.185               | 73.8              |
| Di cresyl dithiophosphoric acid                                   | 1.0                | 0.080               | 88.4              |
| Mixture of Di cresyl dithiophosphoric acid and thiocarbanilide    | 1.0                | 0.076               | 88.9              |
| Mixture of Di cresyl dithiophosphoric acid and di-o-tolylthiourea | 1.0                | 0.078               | 88.7              |
| Ammonium di cresyl dithiophosphate                                | 1.0                | 0.087               | 87.3              |
| Mixture of Ammonium di cresyl dithiophosphate and thiocarbanilide | 1.0                | 0.105               | 84.7              |
| Sodium mercaptobenzothiazole                                      | 1.0                | 0.128               | 81.4              |
| Thiocarbanilide                                                   | 1.0                | 0.085               | 87.6              |
| Di-o-tolylthiourea                                                | 1.0                | 0.086               | 87.3              |
| Mixture of Thiocarbanilide and Fuel Oil No. 2                     | 2.0                | 0.071               | 89.6              |
| Mixture of Di cresyl dithiophosphoric acid and Fuel Oil No. 2     | 2.0                | 0.058               | 91.6              |
| Diethyl dithiophosphoric acid                                     | 1.0                | 0.210               | 69.4              |
| 2-Benzothiazolyl disulfide                                        | 1.0                | 0.102               | 85.2              |
| Morpholine Salt of mercaptobenzothiazole                          | 1.0                | 0.074               | 89.2              |
| Xylenol                                                           | 1.0                | 0.093               | 86.46             |
| o-Amyl phenol                                                     | 1.0                | 0.08                | 88.36             |
| Di(tertiarybutyl)cresol                                           | 1.0                | 0.075               | 89.20             |
| Di amy1 phenol                                                    | 1.0                | 0.069               | 89.96             |
| Nonyl phenol                                                      | 1.0                | 0.068               | 90.39             |
| Cresylic acid                                                     | 1.0                | 0.082               | 88.06             |
| Mixture 46% No. 2 Fuel Oil, 46% cresylic acid, 8% thiocarbanilide | 3.0                | 0.070               | 89.81             |
| Phenol                                                            | 1.0                | 0.143               | 79.18             |

It will be noted that in the case of the phenols, the presence of alkyl carbon atoms is essential as phenol itself gave no useful result. The same is true of diethyl dithiophosphoric acid which was actually worse than the blank.

#### Example 5

An ore from the Gold Coast analyzing 1.01 oz. gold per ton and 0.86% carbon was ground to 74% —200 mesh and portions were cyanided. The results appear in the following table.

| Reagent Used                                                   |                    | Residue Au, oz./ton | Extr. Au, Percent |
|----------------------------------------------------------------|--------------------|---------------------|-------------------|
| Name                                                           | Amt. Used, lb./ton |                     |                   |
| Blank                                                          |                    | 0.105               | 89.6              |
| Mixture of Di cresyl dithiophosphoric acid and thiocarbanilide | 1.0                | 0.093               | 90.8              |
| Sodium mercaptobenzothiazole                                   | 0.5                | 0.060               | 93.1              |
| Di(2-naphthyl)dithiophosphoric acid and thiocarbanilide        | 2.0                | 0.038               | 96.0              |
| Mixture of Di cresyl dithiophosphoric acid and Fuel Oil No. 2  | 2.0                | 0.045               | 95.4              |

**5**  
**Example 6**

An ore from the Gold Coast analyzing 2.43 oz. gold per ton and 0.72% carbon was ground to 74% —200 mesh and portions cyanided. The results appear in the following table.

| Reagent Used                                                 |                          | Residue<br>Au,<br>oz./ton | Extr. Au,<br>Percent |
|--------------------------------------------------------------|--------------------------|---------------------------|----------------------|
| Name                                                         | Amt.<br>Used,<br>lb./ton |                           |                      |
| Blank                                                        |                          | 0.163                     | 93.3                 |
| Mixture of Dicresyldithiophosphoric acid and thiocarbanilide | 1.0                      | 0.103                     | 95.8                 |

This example shows that even in the case of an ore which contains carbon and yet is readily cyanided an improvement is made by the use of a typical reagent of the present invention; although, of course, here the difference is much smaller than with the more refractory ores. In this respect the results are not greatly different from Example 5, which also dealt with an ore which is fairly amenable to cyanidation.

**Example 7**

A Canadian ore analyzing 0.098 oz. gold per ton and 0.97% carbon was ground to 87% —200 mesh and portions cyanided for 48 hours. The results appear in the following table.

| Reagent Used                                                 |                          | Residue<br>Au,<br>oz./ton | Extr. Au,<br>Percent |
|--------------------------------------------------------------|--------------------------|---------------------------|----------------------|
| Name                                                         | Amt.<br>Used,<br>lb./ton |                           |                      |
| Blank                                                        |                          | 0.097                     | 1.0                  |
| Mixture of Dicresyldithiophosphoric acid and thiocarbanilide | 1.0                      | 0.068                     | 30.6                 |
| Mixture of Dicresyldithiophosphoric acid and Fuel Oil No. 2  | 2.0                      | 0.033                     | 66.3                 |

This ore illustrates the fact that with an extremely refractory ore in which ordinary cyanidation gives practically no extraction at all, improvement is obtained and this improvement is greater when the reagents of the present invention are combined with hydrocarbon oils.

**6**  
**Example 8**

Another ore from the Gold Coast analyzing 0.285 oz. gold per ton and 0.38% carbon was ground to 84% —200 mesh and portions cyanided for 48 hours.

| Reagent Used                                                 |                          | Residue<br>Au,<br>oz./ton | Extr. Au,<br>Percent |
|--------------------------------------------------------------|--------------------------|---------------------------|----------------------|
| Name                                                         | Amt.<br>Used,<br>lb./ton |                           |                      |
| Blank                                                        |                          | 0.025                     | 89.9                 |
| Di(2-naphthyl)dithiophosphoric acid                          | 2.0                      | 0.018                     | 92.7                 |
| Mixture of Dicresyldithiophosphoric acid and thiocarbanilide | 2.0                      | 0.019                     | 93.0                 |

This ore which is extremely low in carbon and is amenable to ordinary cyanidation shows that the reagents of the present invention are capable of producing improvement even where so high an extraction can be obtained in ordinary cyanidation procedure.

We claim:

1. A process of extracting cyanidable precious metals from carbonaceous ores containing the same which comprises effecting cyanidation in the presence of an amount of a diaryldithiophosphoric anion having less than twice as many aliphatic carbon atoms as aromatic carbon atoms sufficient to minimize the reprecipitating effect of the carbon and recovering the extracted precious metals.
2. A process according to claim 1 in which the diaryldithiophosphoric anion is dicresyldithiophosphoric anion.
3. A process according to claim 1 in which the diaryldithiophosphoric anion is di(2-naphthyl)dithiophosphoric anion.
4. A process according to claim 1 in which the cyanidation agent is an alpha-hydroxynitrile.
5. A process according to claim 4 in which the alpha-hydroxynitrile is crude lactonitrile.

**References Cited in the file of this patent**

**FOREIGN PATENTS**

45 554,290 Great Britain June 28, 1943